

Dec. 21, 1948.

E. F. PINNEY

**2,457,088**

## METHOD FOR THE PRODUCTION OF CANDLES

Filed Sept. 26, 1945

3 Sheets-Sheet 1



## INVENTOR

ERNEST F. PINNEY  
BY  
Myron J. Bushard  
AGENT OR ATTORNEY

Dec. 21, 1948.

E. F. PINNEY

2,457,088

METHOD FOR THE PRODUCTION OF CANDLES

Filed Sept. 26, 1945

3 Sheets-Sheet 2

Fig. 3,



Fig. 2,



Fig. 4,



INVENTOR

ERNEST F. PINNEY

BY

*George F. Bushnell*  
AGENT OR ATTORNEY

Dec. 21, 1948.

E. F. PINNEY

2,457,088

METHOD FOR THE PRODUCTION OF CANDLES

Filed Sept. 26, 1945

3 Sheets-Sheet 3

FIG. 5



INVENTOR.  
ERNEST F. PINNEY

BY

*Myron J. Burkhead*

ATTORNEY

## UNITED STATES PATENT OFFICE

2,457,088

METHOD FOR THE PRODUCTION  
OF CANDLES

Ernest F. Pinney, Glen Cove, N. Y., assignor to  
Socony-Vacuum Oil Company, Incorporated,  
New York, N. Y., a corporation of New York

Application September 26, 1945, Serial No. 618,767

2 Claims. (Cl. 18—55)

1

One of the oldest arts in the world is that of candle making. Similarly it is one in which probably the least modernization has occurred. The major changes around the first of this century passed from hand dipping or molding in single hand filled molds to a method of molding entirely similar in its essentials to the old hand method except that it was executed in multiple molds capable of producing a large number of candles, ranging from several dozen to several gross, dependent upon the size of the candle.

This invention has to do with a new and improved method of making candles particularly suitable for the manufacture of a large number of candles at a low production cost.

The invention is based upon the concept of extrusion, that is, a candle stock mixture is reduced from a liquid to a plastic condition and extruded through a die to form a continuous candle rod, which candle rod is later severed into lengths to form candles of commerce.

The mechanical setup of the invention may be readily understood by reference to the drawings attached to this specification. In these drawings, Figure 1 shows a general view, partially in section, of the candle forming machine. Figure 2 is a detail of the method of drive therefor, as is Figure 3, and Figure 4 shows the essential details in section of the die and associated parts which are the essential candle forming mechanism. Figure 5 is a highly diagrammatic showing of the entire operating setup.

Turning now to Figure 1, we find shown therein a supply tank 5 wherein a liquid candle stock mixture is stored, to pass downwardly into a series of heat exchange tubes 6, 6 and 6, exactly similar to the conventional Carbondale and other wax chillers used in the paraffin recovery practice of the oil industry. Each heat exchanger consists of an inner pipe 7 surrounded by a jacket 8 to which cooling material is supplied, as by pipe 9. These inner tubes, through which the candle mixture flows to be chilled, are connected serially by return bends, as is shown quite clearly in the drawing. Each cooling tube has mounted inside of it a helical scroll or scraper blade 10 carried by a shaft 11, which shaft is supported upon proper outboard bearings 12, 12 at either end of the heat exchanger tube. These scrapers are driven by a chain mechanism later explained in detail, and their direction of rotation is such that in rotating they tend to force the plastic mass to which candle stock mixture is chilled through the serially connected cooling tubes, imposing thereupon sufficient pressure to force it out of the

2

end of the chillers and through the forming die. Not only do these scrapers accomplish this function of moving the material through the chilling apparatus, but of equal and possibly of more importance, they keep the interior walls of the heat exchanger tubes freed from the deposit of wax formed other than by the chilling and so keep the rate of heat exchange in the chiller constant.

The scraper mechanism in the upper exchanger 10, tube 6 and the middle exchanger tube 6, is the same except for directional function. However, in the lower tube of the three a change is made.

In this tube, shaft 13 carrying scraper 14 is hollow, and while it is supported by an outboard bearing 12 at the left hand or entry end of the tube in which it is placed, this shaft and its accompanying scraper terminate short of the discharge end of the tube and are carried internally upon bearings 15 supported in a proper spider situated internally of the cooling tube. A second shaft 16 extends throughout the length of the hollow shaft 14, is driven upon its drive end by a separate drive at 17, is supported within the right hand extremity of the lowermost cooling tube by another internal spider, not shown, and carries in the space between this last named bearing and the end of shaft 13 a scraper or scroll 18. This scraper or scroll 18 is so mounted upon the shaft that while its rotation serves to advance the plastic material which the candle stock has now become in the same direction, its rotation is counter to the direction of rotation of scroll 14, and preferably its pitch is quite different from that of scroll 14. This change in construction is made to insure complete mixing of the plastic candle stock prior to its exit from the chilling stage of the operation. The chiller is equipped with a cutoff valve 19 at its discharge end with a candle forming die 20 which is later explained and with a wick supply spool 21.

Turning to Figures 2 and 3 and reading them in connection with Figure 1, we find the drive mechanism for this chiller to be as follows:

A motor 22 through a chain 23 and a gear and a speed reducer 24 drives chain 25. Chain 25 acting through sprocket wheel 26, keyed upon the outboard extension of shaft 13, in turn actuates sprocket wheel 27, which is also keyed to shaft 13 and chain 28 passing thereover as is shown in Figure 3 actuates successively sprocket wheels 29 and 30, each of which is keyed to the shaft mounted within another chilling tube, returning finally over idler 31. This arrangement is conventional for chillers of this type, except as to matters of speed choice which are dependent upon

the heat transfer characteristics of the chiller and physical nature of the mixture being handled and may be selected as is well known within the art. In order to provide for the drive of the mixer section 18 near the terminal of the chiller, the shaft in that chilling tube next above the terminal chilling tube which shaft rotates in a direction opposite to that in the terminal chilling tube, is extended at its outboard end to support and drive sprocket wheel 32, (Figures 1 and 2), which sprocket wheel through chain 33 drives sprocket wheel 17 which is keyed upon the outboard end of shaft 16 which supports scroll 18.

Turning now to Figure 4, we find an explanation of the mechanism through which the extruded candle is formed. Mounted upon the outboard valve 19 at the terminal end of the chiller, there is a flange 34 supporting a tapered cone 35 which ends in a die ring 36 of the size to which the candle is to be made. Forced by the internal scrolls in the chiller, the plastic candle stock is forced through this cone and die and exits therefrom in the form of a cylindrical rod. To assist in the formation of the candle and in particular to provide a finish upon its surface, a cylindrical "polish tube" 37 having an internal diameter equal to the external diameter of the finished candle and ranging in length from about one foot to several feet, depending upon the exact size of the finished candle, is affixed into the end of the die cone 35. A wick 38 is centrally disposed within the candle as it is extruded by any one of several suitable mechanisms, the simplest of which is that shown in Figure 4, consisting of a bent tube 39 extending through the wall of cone 35 bending into the flow of the plastic mass and terminating upon the center line thereof, so that the wick 38 may be withdrawn therethrough and positioned centrally within the candle rod as it is extruded. Another, and possibly a better way, of introducing the wick is to provide for, as shaft 16, (see Figure 1), a centrally drilled tube and to feed the wick into the candle throughout the length of this tube.

Upon extrusion, the candle rod passes into trough 40 in which there is maintained a supply of water 41 for the purpose hereinafter explained.

In Figure 5 there is a diagrammatic showing of the entire operating setup. Here there is shown the supply tank 15, the chiller 6, valve 19, the die tube 35, wick 38 coming from wick supply 21, and candle rod 42 passing from the die into chiller trough 40. Emerging from the opposite end of trough 40 the candle rod 42 passes over table 43, is severed, as by reciprocating knife or other severing means 44, and the severed end is removed to further processing by conveyor 45.

The mere utilization of the mechanical setup hereinbefore explained is not sufficient to produce good candles without proper control of the variables present. For example, the temperature at which the candle stock mix arrives just prior to the point of extrusion is an important variable in the process. The stock must be at a temperature sufficiently far below its melting point to assure that the candle when formed is sufficiently strong physically to be handled in the subsequent cooling trough without substantial kinking or bending or deformation of its surface. Yet the candle stock must not be too far chilled because then it will not only require larger amounts of power for handling, but will give a much less satisfactory candle and one which exhibits surface tear and pitting and other imperfections. In general, the proper temperature

for extrusion will be found to range from 8° F. to 20° F. below the melting point (American melting point) A. S. T. M. method. Other important details center around the handling of the candle rod in the cooling trough 40. Only a small portion of one end of this cooling trough is shown in the drawing. In practice it is of considerable length, usually about 40 feet long and the cooling of the candle rod therein is divided into two stages. First, a tempering stage and second, a hardening stage.

The candle rod when extruded, and not subjected to further treatment, is found to have several undesirable features. Probably the most pronounced of these is a longitudinal crystalline structure, almost fibrous in nature, coupled with what might be termed a "case-hardened" condition at the surface of the rod. This condition leads to extremely erratic burning of the candle. For example, a 1 1/4" diameter candle 5" long, formed without tempering, will usually burn rather decently for the first two inches or so of its length. After that as the heat of the flame works its way downwardly into the body of the candle, the difference in crystalline structure apparently results in a melting of the interior of the candle long before the exterior shell of the candle melts with a resulting pressure effect of some kind or another which usually ends in the candle "blooming," that is, expanding into a structure rather resembling the flower of the well known calla lily, with one or more breaks in the outwardly flaring walls of the candle through which molten material escapes, the whole resulting in a practical uselessness of about half of the length of the original candle. A properly tempered candle on the other hand will burn almost completely without essential change in its burning characteristics after it has once been well started.

This tempering is achieved by maintaining within the first portion of the cooling trough, that is within the tempering portion, a bath of water which is at from about 15° F. to about 40° F. below the melting point of the candle stock mixture. It has been found that the time during which the candle should be tempered, which depends upon the diameter of the candle, is about 1/2 to 1 1/2 minutes. Having determined the rate at which a candle rod is extruded, this determines the length of the tempering section of trough 40.

The cooling section of trough 40 is much simpler in concept and merely consists of a portion through which water is flowed at a temperature sufficiently low with respect to the length of the trough to harden the candle rod so that it will stand subsequent handling.

While two functional sections of trough 40 have been described, there is no necessity for a major physical division into two troughs. It is sufficient merely to elevate the bottom of the trough slightly near the point of division so that a major flow of the water in either section is away from this point of division towards either end and a major amount of mixing of the two baths will not occur or at least not sufficient to trouble proper operation. At the delivery end of trough 40, the bottom of the trough may be brought up on a slope to raise the rod above the water, or a conveyor, motor driven, synchronized with rate of extrusion may be installed at end of trough 40 to convey candle rod to a following cutting unit.

The operation and apparatus above described have achieved the production of a continuous candle rod. This rod is then severed into lengths,

as shown in my copending applications Serial Number 618,770, and Serial Number 618,768, both filed September 26, 1944, (the latter now being abandoned), and tipped as shown in my application Serial Number 618,769, now U. S. Patent 2,415,369.

I claim:

1. That method for the production of candles which comprises flowing a liquid candle stock melt into a chiller and advancing it therethrough while chilling it to a plastic condition, mixing and extruding the chilled plastic stock from said chiller through a candle rod forming die, disposing a wick in said stock prior to extrusion so that it will extend axially of the candle rod formed by extrusion, passing the candle rod through a first controlled cooling at a temperature of from about 15° F. to about 40° F. below the melting point of the stock, said first cooling step being of a duration of from about  $\frac{1}{2}$  to 1  $\frac{1}{2}$  minutes and sufficient to permit adjustment of its internal structure to a substantially non-oriented crystal arrangement and then through a second cooling step to harden it to a point where it will withstand mechanical handling, and severing the continuously extruded rod into desired lengths.

2. That method for the production of candles which comprises flowing a liquid candle stock melt into a chiller and advancing it therethrough while chilling it to a plastic condition, at a tem-

perature of from about 8° F. to about 20° F. below the melting point of the stock, mixing and extruding the chilled plastic stock from said chiller through a candle rod forming die, disposing a wick in said stock prior to extrusion so that it will extend axially of the candle rod formed by extrusion, passing the candle rod through a first controlled cooling to a temperature of from about 15° F. to about 40° F. below the melting point of the stock, said first cooling step being of a duration of from about  $\frac{1}{2}$  to about 1  $\frac{1}{2}$  minutes and sufficient to permit adjustment of its internal structure to a substantially non-oriented crystal arrangement and then through a second cooling step to harden it to a point where it will withstand mechanical handling, and severing the continuously extruded rod into desired lengths.

ERNEST F. PINNEY.

#### REFERENCES CITED

The following references are of record in the file of this patent:

#### UNITED STATES PATENTS

| Number    | Name       | Date          |
|-----------|------------|---------------|
| 1,294,008 | Will       | Feb. 11, 1919 |
| 1,312,424 | Richardson | Aug. 5, 1919  |
| 1,361,346 | Nichols    | Dec. 7, 1920  |
| 1,571,589 | Kerr       | Feb. 2, 1926  |